

March 28, 1967

C. R. LOPER, JR., ETAL

3,311,469

MANUFACTURE OF NODULAR IRON

Filed April 23, 1964



## 1

3,311,469

**MANUFACTURE OF NODULAR IRON**  
Carl R. Loper, Jr., and Richard W. Heine, both of Madison, Wis., assignors, by mesne assignments, to Union Carbide Corporation, a corporation of New York  
Filed Apr. 23, 1964, Ser. No. 362,056  
2 Claims. (Cl. 75—130)

The present invention relates to the manufacture of nodular iron. More particularly, the present invention relates to an improved process for increasing the proportion and amount of truly spheroidal graphite in nodular irons.

In the production of nodular iron castings, to obtain a high quality product, it is required that, during the solidification of the iron, an adequate number of graphite spheroids be nucleated and caused to grow uniformly as solidification progresses in order to depress the formation of carbides and undesirable graphitic shapes such as vermicular graphite.

In the past, in efforts to achieve this effect, magnesium has been used as an addition to induce the formation of spheroidal graphite and silicon has been used as a graphitizing inoculant. However, in the use of these materials, metal temperature and the carbon equivalent (C=percent C+1/3% Si) and carbon contents of the base metal have had to be rather closely controlled. Moreover, even using very closely controlled processing conditions, the results have not been entirely successful as regards the total amount of truly spheroidal graphite produced, the elimination of undesirable vermicular graphite, and the prevention of carbide formation.

It is therefore an object of the present invention to provide a process for the production of nodular iron in which the amount of spheroidal graphite is substantially increased.

It is another object of the present invention to provide a process which substantially eliminates the presence of carbides in nodular iron.

It is a further object of the present invention to provide a process whereby vermicular graphite is substantially eliminated from nodular iron.

It is another object of the present invention to provide a process which permits the use of lower temperatures in the casting of nodular iron.

It is a further object of the present invention to provide a process which permits lower carbon equivalent irons, e.g., 4.3—4.4, to be cast without the formation of vermicular graphite or carbides.

Other objects will be apparent from the following description and claims in conjunction with the drawing which graphically and comparatively illustrates advantages of the present invention.

A process in accordance with the present invention to achieve the aforementioned objects comprises bringing together molten iron, magnesium and bismuth.

In the practice of a particular embodiment of the present invention, a bath of molten iron containing from

## 2

about 3.5 to 5.0% carbon equivalent is prepared and to this iron bath is added magnesium, for example in the form of magnesium-ferrosilicon, and bismuth, which can conveniently be in lump form. A practical manner of making the magnesium and bismuth addition is to place the magnesium-ferrosilicon and bismuth in a pocket at the bottom of a ladle and pouring molten iron onto the material in the pocket. Subsequently, the thus treated molten iron can be transferred to a pouring ladle and ultimately cast into suitable shapes.

In the present invention, the molten iron should contain from about 3.5 to about 5.0% carbon equivalent, which can derive partly by way of the ferrosilicon addition. This carbon equivalent is necessary in order to produce a spheroidal graphite cast iron which will graphitize during solidification.

Silicon in an amount from about 1% to 5% should also be present in the base iron in order to cause graphite formation. The silicon can be initially present in the base metal or it can be added wholly or partly in the form of ferrosilicon inoculant following conventional practice.

The magnesium addition should range from about 0.02 to 0.25% by weight of the iron and the bismuth addition ranges from very small amounts, sufficient to provide an increase in spheroidal graphite, up to 0.1%.

As little as 0.0001% bismuth addition will provide a substantial increase in the amount of spheroidal graphite compared to the amount produced using magnesium without bismuth.

An industrially convenient range for the bismuth addition to provide significant advantages is from 0.0005% to 0.050%, a preferred range for the bismuth addition is from about 0.01% to about 0.015%.

In order to demonstrate the effectiveness of bismuth as an addition in the manufacture of nodular iron, various tests were performed as hereinafter described.

The metal used in the tests was commercial iron and was melted in a basic cupola. A 1500 lb. mixing ladle was arranged in front of the cupola and 150 lb. transfer ladles, having a pocket in the bottom, were also provided.

Treatment of the base metal involved placing a predetermined amount of magnesium-ferrosilicon (46.99% Si, 0.78% Al, 9.49% Mg, 0.53% Ce) in the pocket at the bottom of a ladle and covering it with ferrosilicon inoculant (48.79% Si). Base iron in the amount of 750 lbs. was poured onto the material in the pocket.

The metal in the ladle was cleaned of dross and the treated iron was transferred to 250 lb. covered pouring ladles. Approximately two minutes elapsed from the time of treatment of the base metal to the transfer into the pouring ladles. After various holding times, the metal was poured at predetermined temperatures into molds and sample castings were prepared. Analysis data for the metal tested is shown in Table I together with pouring temperatures and holding times.

The holding times shown in Table I start from the time the pouring ladles were filled.

TABLE I.—LADLE DATA SHOWING CHEMICAL ANALYSIS, POURING TEMPERATURE, AND PERCENT MAGNESIUM SILICON, AND OTHER ADDITIONS ADDED.

[Asterisk (\*) denotes estimated values.]

| Ladle No. | Analysis, <sup>3, 4</sup> percent |                 |          |       | Pouring Temp., °F. | Holding Time, Min:Sec | Percent Mg Added as Mg-Fe-Si | Percent Mg Recovered | Percent Si Added |          | Percent Other Additions |
|-----------|-----------------------------------|-----------------|----------|-------|--------------------|-----------------------|------------------------------|----------------------|------------------|----------|-------------------------|
|           | C (pin)                           | C (bar)         | Si (bar) | C.E.  |                    |                       |                              |                      | As Mg-Fe-Si      | As Fe-Si |                         |
| B-1       | 3.97                              | 4.05            | 2.13     | 4.76  | 2,700              | 0                     | 0.280                        | 0.076                | 1.387            | 0.245    | 0.                      |
| B-2       | 3.92                              | NR <sup>1</sup> | 2.14     | *4.76 | 2,420              | 23:40                 | 0.280                        | 0.047                | 1.387            | 0.245    | 0.                      |
| B-3       | 3.51                              | 3.50            | 2.12     | 4.21  | 2,580              | 0                     | 0.280                        | 0.074                | 1.387            | 0.245    | 0.                      |
| B-4       | 3.56                              | NR <sup>1</sup> | 2.18     | *4.29 | 2,300              | 15:30                 | 0.280                        | 0.072                | 1.387            | 0.245    | 0.                      |
| B-5       | 3.70                              | 3.56            | 2.05     | *4.33 | 2,560              | 0                     | 0.280                        | 0.067                | 1.387            | 0.245    | 0.                      |
| B-6       | 3.73                              | NR <sup>1</sup> | 2.10     | *4.43 | 2,300              | 16:00                 | 0.280                        | 0.064                | 1.387            | 0.245    | 0.                      |
| B-7       | 3.65                              | 3.52            | 2.00     | *4.32 | 2,570              | 0                     | 0.130                        | 0.048                | 0.640            | 0.956    | 0.014 Bi. <sup>2</sup>  |
| B-8       | 3.71                              | 3.61            | 2.10     | 4.31  | 2,290              | 14:00                 | 0.130                        | 0.041                | 0.640            | 0.956    | 0.014 Bi. <sup>2</sup>  |

<sup>1</sup> NR=not reported.<sup>2</sup> Bismuth added in lump form.<sup>3</sup> Pin samples for carbon analyses taken from the ladle.  $\frac{1}{2}$  in. diameter bars used for C analyses.  $\frac{1}{2}$  in. diameter bars used for Si analyses. Carbon equivalent percentage=percent C+ $\frac{1}{8}$  percent Si.<sup>4</sup> Typical amounts of other elements are as follows:

|    |       |                 |        |    |         |
|----|-------|-----------------|--------|----|---------|
| S  | 0.012 | Mg              | 0.04   | Sn | 0.01    |
| P  | 0.022 | Tl              | 0.009  | As | 0.01    |
| Mn | 0.36  | Pb              | <0.003 | P  | 0.015   |
| Ni | 0.02  | Bi <sup>1</sup> | <0.005 | B  | <0.0005 |
| Mo | 0.03  | Sb              | <0.005 | Cr | 0.09    |
| Cu | 0.12  | Al              | 0.01   |    |         |

<sup>a</sup> Except B-7 and B-8.

The castings obtained following the aforescribed procedure were examined with regard to nodule count, nodule size, graphite type and presence of carbides.

Nodule counts were obtained by projecting an image of the specimen on a ground glass screen using an 8.0 x 0.20 Na objective lens; a 10 $\times$  hyperplane eyepiece; and adjusting to obtain a magnification of 200 $\times$ . The number of graphite nodules greater than  $\frac{1}{16}$  inch diameter on the ground glass screen was then determined in a 10 cm. x 10 cm. area. Four random counts were made and added to obtain the number of nodules per mm.<sup>2</sup> of sample surface area. Nodule sizes were recorded by measuring their diameter on the ground glass screen at 200 $\times$  and converting them to actual nodule dimensions.

Graphite type was recorded as spheroidal, compact and vermicular. Spheroidal graphite is essentially spherical

and is readily identifiable visually at magnifications of say 55 $\times$ ; compact graphite refers to those shapes which deviate from spheroidal by being ragged and irregular; and vermicular graphite refers to shapes varying from short stubby graphite to more worm-like graphite shapes.

Carbide formation in the cast samples was observed visually.

The results of the aforescribed observations are summarized in Tables II, III and IV. Tables VI, VII and the drawing show the test results obtained by preparing additional castings, with and without bismuth additions, following substantially the same procedure as described hereinabove.

The nodule counts in the tables includes spheroidal, compact and vermicular shapes.

TABLE II.—SUMMARY OF DATA FOR 1.0 INCH DIAMETER BAR CASTING

| Ladle No. | Nodule Count <sup>a</sup> per mm. <sup>2</sup> |        |      | Nodule Size, <sup>b</sup> mm. $\times 10^{-2}$ |          |      | Graphite Shape, Percent |         |            | Carbides <sup>c</sup> |
|-----------|------------------------------------------------|--------|------|------------------------------------------------|----------|------|-------------------------|---------|------------|-----------------------|
|           | Cope                                           | Center | Drag | Cope                                           | Center   | Drag | Spheroids               | Compact | Vermicular |                       |
| B-1       | 150                                            |        |      | 154                                            | 1/2+4+11 |      | 90                      | 10      |            | 0 CLC.                |
| B-2       | 162                                            |        |      | 163                                            | 1/2+7/9  |      | 90                      | 10      |            | 0 CAS.                |
| B-3       | 159                                            |        |      | 120                                            | 1/2+4/5  |      | 90                      | 10      |            | 0 CAS.                |
| B-4       | 181                                            |        |      | 128                                            | 1/2+3    |      | 80                      | 20      |            | 0 CAS.                |
| B-5       | 174                                            |        |      | 161                                            | 1+2      |      | 90                      | 10      |            | 0 CAS.                |
| B-6       | 152                                            |        |      | 125                                            | 1+4      |      | 90                      | 15      |            | 0 CAS.                |
| B-7       | 314                                            |        |      | 288                                            | 1+4/7    |      | 85                      | 0+      |            | 0 NC.                 |
| B-8       | 318                                            |        |      | 269                                            | 1+4      |      | 100                     | 10      |            | 0 CAS.                |

See footnotes at end of table V.

TABLE III.—SUMMARY OF DATA FOR 1.5 INCH DIAMETER BAR CASTING

| Ladle No. | Nodule Count <sup>a</sup> per mm. <sup>2</sup> |        |      | Nodule Size, <sup>b</sup> mm. $\times 10^{-2}$ |         |      | Graphite Shape, Percent |         |            | Carbides <sup>c</sup> |
|-----------|------------------------------------------------|--------|------|------------------------------------------------|---------|------|-------------------------|---------|------------|-----------------------|
|           | Cope                                           | Center | Drag | Cope                                           | Center  | Drag | Spheroids               | Compact | Vermicular |                       |
| B-1       | 94                                             |        |      | 104                                            | 2+3/6   |      | 80                      | 20      |            | 0 NC.                 |
| B-2       | 93                                             |        |      | 64                                             | 2/3+8   |      | 80                      | 20      |            | 0 CLC.                |
| B-3       | 51                                             |        |      | 56                                             | 4/9     |      | 2/9                     | 50      |            | 0 CAS.                |
| B-4       | 90                                             |        |      | 118                                            | 1/2+9   |      | 20                      | 75      | 5          | 0 CAS.                |
| B-5       | 88                                             |        |      | 86                                             | 2+4/8   |      | 4/8                     | 60      | 40         | 0 CAS.                |
| B-6       | 108                                            |        |      | 91                                             | 1/2+4   |      | 2/13                    | 20      | 75         | 5 CAS.                |
| B-7       | 130                                            |        |      | 132                                            | 1/2+3/4 |      | 1/2+3/4                 | 85      | 15         | 0 NC.                 |
| B-8       | 172                                            |        |      | 132                                            | 1+4     |      | 1/2+4                   | 50      | 50         | 0 Trace.              |

See footnotes at end of table V.

TABLE IV.—SUMMARY OF DATA FOR 2.0 INCH DIAMETER BAR CASTING

| Ladle No. | Nodule Count <sup>a</sup> per mm. <sup>2</sup> |        |      | Nodule Size, <sup>b</sup> mm. $\times 10^{-2}$ |        |         | Graphite Shape, Percent |         |            |                       |
|-----------|------------------------------------------------|--------|------|------------------------------------------------|--------|---------|-------------------------|---------|------------|-----------------------|
|           | Cope                                           | Center | Drag | Cope                                           | Center | Drag    | Spheroids               | Compact | Vermicular | Carbides <sup>c</sup> |
| B-1       | 78                                             |        | 106  | 1+3/11                                         |        | 3/8     | 75                      | 25      | 0          | NC.                   |
| B-3       | 47                                             |        | 48   | 3/9                                            |        | 1/2+6/8 | 20                      | 80      | 0          | NC.                   |
| B-4       | 104                                            |        | 114  | 1/2+4/9                                        |        | 1/2+4/9 | 10                      | 85      | 5          | CAS.                  |
| B-5       | 99                                             |        | 107  | 1+4/13                                         |        | 1+4/9   | 20                      | 75+     | 5          | NC.                   |
| B-6       | 101                                            |        | 106  | 1/2+4/9                                        |        | 1/2+4/9 | 10                      | 80      | 10         | CAS.                  |
| B-7       | 144                                            |        | 156  | 1+3/9                                          |        | 1+3/9   | 85                      | 15      | 0          | NC.                   |
| B-8       | 135                                            |        | 141  | 1+3/6                                          |        | 1+3/6   | 40                      | 60      | 0          | NC.                   |

See footnotes at end of Table V.

TABLE V.—SUMMARY OF DATA FOR THE 2.5 INCH DIAMETER BAR

| Ladle No. | Nodule Count <sup>a</sup> per mm. <sup>2</sup> |        |      | Nodule Size, <sup>b</sup> $\frac{1}{16}$ " units at 200X |        |       | Graphite Shape, Percent |         |            |                       |
|-----------|------------------------------------------------|--------|------|----------------------------------------------------------|--------|-------|-------------------------|---------|------------|-----------------------|
|           | Cope                                           | Center | Drag | Cope                                                     | Center | Drag  | Spheroids               | Compact | Vermicular | Carbides <sup>c</sup> |
| B-1       | 54                                             |        | 39   | 3+11                                                     |        | 3+11  | 50                      | 50      | 0          | NC.                   |
| B-3       | 47                                             |        | 46   | 3+9                                                      |        | 2+9   | 20                      | 80      | 0          | NC.                   |
| B-4       | 65                                             |        | 48   | 1+8                                                      |        | 1/2+9 | 5                       | 75      | 20         | CAS.                  |
| B-5       | 57                                             |        | 51   | 1/2+9                                                    |        | 1/2+9 | 20                      | 80      | 0          | NC.                   |
| B-6       | 69                                             |        | 57   | 3/7                                                      |        | 3/7   | 15                      | 75      | 10         | CLC.                  |
| B-7       | 89                                             |        | 115  | 2/7                                                      |        | 2+4   | 85                      | 15      | 0          | NC.                   |
| B-8       | 73                                             |        | 79   | 4/9                                                      |        | 3/9   | 50                      | 50      | 0          | NC.                   |

<sup>a</sup>Nodule counts include all graphite shapes over  $\frac{1}{16}$  inch diameter when viewed at 200X.<sup>b</sup>Nodule size is represented by values indicating the approximate diameter of the graphite shape. A value of 2/6 is read as diameters ranging from 2 to 6. A value of 2+4 indicates two separate sizes of graphite shapes.<sup>c</sup>Designations in carbides column are read as follows:

NC=No carbides.

Trace=Trace of carbides at center.

CLC=Centerline carbides.

C1/2R=Carbides in center 1/2 radius.

C2/3R=Carbides in center 2/3 radius.

CAS=Carbides across section.

TABLE VI (refer to drawing).—EFFECT OF ADDITION, POURING TEMPERATURE AND SECTION SIZE ON PERCENTAGE OF EACH GRAPHITE SHAPE

| Chemical Analysis | Bar Diam. (in.)            | 0.14% Mg Added               |                               | 0.14% Mg Added plus 0.01% Bi Added |                               | 0.28% Mg Added               |                               |
|-------------------|----------------------------|------------------------------|-------------------------------|------------------------------------|-------------------------------|------------------------------|-------------------------------|
|                   |                            | Poured Hot (2,515-2,700° F.) | Poured Cold (2,300-2,475° F.) | Poured Hot (2,515-2,700° F.)       | Poured Cold (2,300-2,475° F.) | Poured Hot (2,515-2,700° F.) | Poured Cold (2,300-2,475° F.) |
| 4.31-4.43% C.E.   | { 1.0<br>1.5<br>2.0<br>2.5 | Figure 1                     | Figure 2                      | Figure 3                           | Figure 4                      | Figure 5                     | Figure 6                      |

TABLE VII.—EFFECT OF ADDITIONS, POURING TEMPERATURE, AND SECTION SIZE ON CARBIDE FORMATION\*

| Chemical Analysis | Bar Diam. (in.)            | 0.14% Mg Added <sup>1</sup>  |                               | 0.14% Mg Added plus 0.015% Bi Added |                               | 0.28% Mg Added <sup>1</sup>  |                               |
|-------------------|----------------------------|------------------------------|-------------------------------|-------------------------------------|-------------------------------|------------------------------|-------------------------------|
|                   |                            | Poured Hot (2,515-2,700° F.) | Poured Cold (2,300-2,475° F.) | Poured Hot (2,515-2,700° F.)        | Poured Cold (2,300-2,475° F.) | Poured Hot (2,515-2,700° F.) | Poured Cold (2,300-2,475° F.) |
| 4.31-4.43% C.E.   | { 1.0<br>1.5<br>2.0<br>2.5 | CLC                          | CAS                           | NC                                  | CAS                           | CAS                          | CAS                           |

<sup>1</sup>Nominal amounts.

\*Designations for carbide formation are as follows:

NC=No carbides.

C1/2R=Carbides in center 1/2 radius.

Trace=Trace of carbides at center.

C2/3R=Carbides in center 2/3 radius.

CLC=Centerline carbides.

CAS=Carbides across section.

As can be seen from the data in the tables, the metal treated with bismuth in accordance with the present invention (B7 and B8) exhibit an overall superiority as compared to the other irons.

For example, the bismuth treated iron, as shown in Tables II-V have, on the average, 50 to 100% more nodules than the other irons. Also, as shown in Tables II-V, carbide formation and vermicular graphite are essentially eliminated from the bismuth treated irons.

Table VI in conjunction with the drawing further graphically illustrates that bismuth treated irons can be poured "cold" and provide, on the average, higher amounts of spheroidal graphite. The advantage of the bismuth treatment is particularly pronounced for the larger diameter castings.

Table VII further illustrates that iron treated with bis-

60 muth in accordance with the present invention can be poured "cold" without the formation of a deleterious amount of carbides.

The overall effect of the changes in the microstructure of iron castings by bismuth treatment as aforescribed results in the production of nodular irons having substantially improved mechanical properties. The as-cast microstructure is improved as follows:

(a) vermicular graphite and other undesirable graphite shapes such as flakes are substantially eliminated from the as-cast microstructure.

(b) the number of graphite spheroids per unit volume of iron is increased

(c) carbides are substantially prevented due to the increased number of graphite spheroids precipitated.

Further, irons of 4.3 carbon equivalent and under can be cast substantially without the formation of undesirable graphite shapes and undesirable graphite shapes and carbides are avoided even in larger casting section thicknesses.

What is claimed is:

1. In a process for making nodular iron by bringing together magnesium, silicon and molten iron, the improvement which comprises providing in the molten iron a silicon content of between about 1 to 5%, a magnesium addition of about 0.02 to 0.25% and a bismuth addition of from about 0.010 to about 0.050%, said bismuth addition being sufficient to provide a substantial increase in the amount of spheroidal graphite nodules in the iron as compared to the same iron without a bismuth addition.

2. An improved process in accordance with claim 1

wherein the bismuth addition is in the range of about 0.010 to about 0.015%.

**References Cited by the Examiner**

**UNITED STATES PATENTS**

|    |           |         |                |       |          |
|----|-----------|---------|----------------|-------|----------|
| 5  | 2,485,760 | 10/1949 | Millis et al.  | ----- | 75—130   |
|    | 2,536,204 | 1/1951  | Morrogh et al. | ----- | 75—130 X |
|    | 2,579,452 | 12/1951 | Eckman et al.  | ----- | 75—130 X |
| 10 | 2,780,541 | 2/1957  | Zifferer       | ----- | 75—130   |
|    | 2,841,490 | 7/1958  | Steven         | ----- | 75—130   |
|    | 2,943,932 | 7/1960  | White et al.   | ----- | 75—130 X |

DAVID L. RECK, *Primary Examiner.*  
15 HYLAND BIZOT, H. W. TARRING,  
*Assistant Examiners.*